

## UNITED STATES PATENT OFFICE

2,025,425

## STEEL MAKING PROCESS

Earl C. Smith, Canton, Ohio, assignor to Republic Steel Corporation, Youngstown, Ohio, a corporation of New Jersey

No Drawing. Application April 18, 1935,  
Serial No. 17,138

4 Claims. (Cl. 75—48)

This invention relates to the manufacture of steel, and particularly to a method of controlling the abrasiveness of non-metallic substances in steel.

5 Highly abrasive non-metallic substances are usually present in steels produced by present day methods. When a steel containing such substances is machined, these substances quickly dull and wear the cutting tools so that the life of such 10 tools is short.

I have found that the degree of abrasiveness of such substances can be greatly reduced with coincident prolongation of cutting tool life. The reduction I have accomplished has increased the 15 cutting tool life by 100% or more without any attendant disadvantages.

The present invention is predicated on the discovery that the abrasiveness of non-metallic substances normally formed by chemical reactions in 20 the molten steel during its manufacture, is traceable largely to the amount and form of manganese and associated non-metallic manganese compounds present in the steel; and on the discovery that alteration of the form of such manganese 25 and manganese compounds will result in a change in the degree of abrasiveness of the non-metallic substances in the steel.

Briefly described, the present invention includes the steps of making molten steel in any 30 suitable manner, determining the approximate composition of the steel and substances therein, and the nature and amounts of non-metallic forming ingredients, particularly manganese and associated metallic compounds in the steel, and 35 treating the steel in a manner to give the desired properties to the non-metallic substances in the steel.

The present invention will be better understood 40 by those skilled in the art by the following examples in which it may be practiced.

Steel to be machined was made by the usual Bessemer practice. It contained the usual amounts of impurities including sulphur, phosphorus, as well as non-metallic substances such 45 as silicates, the approximate amounts of which were known, and about .05% of manganese in metallic and non-metallic form. About 1.25% of manganese, in the form of ferromanganese, was added in solid form to the steel during pouring 50 and when the ladle was about one-quarter filled with steel. During pouring, and preferably just after the manganese had been added, about 4 pounds of siderite ( $FeCO_3$ ) per ton of steel was thrown into the ladle, the pouring being continued until the ladle was filled. The siderite

evidently decomposed, liberating oxygen or an oxygen containing gas. The metal in the ladle was violently agitated and gas was evolved, and the resulting steel was relatively free from abrasive, non-metallic substances as measured by cutting tool life which was more than double 5 the life obtained on similar steel made in the same way except for the addition of the siderite.

The content of manganese in metallic and non-metallic forms, in the steel of the foregoing example before the addition of the ferromanganese was, as stated, about .05%, and after treatment with the siderite was about .90%. If no siderite or equivalent material had been added the manganese content would have been about 1.00%. 10 Thus the present process tends to remove some 15 of the manganese which would otherwise remain in the steel. This tendency is important, for if it be disregarded difficulty in finishing a steel within the limits of manganese specified may be 20 encountered, particularly in open hearth steels 25 high in manganese.

The amount of siderite or its equivalent which should be used in my method will vary somewhat with the manganese desired in the finished 25 steel. For example, the variation per ton of steel is on about the order of 4 pounds of siderite for .80% of manganese, 7 pounds for 1.00% of manganese and 10 pounds for 1.50% of manganese. 30

It is important to determine the amount of manganese in the steel in metallic and non-metallic forms as a preliminary to determination of the amount of siderite or its equivalent to use. If too small an amount of siderite is used, 35 the degree of abrasiveness of the non-metallic substances will not be greatly decreased, while if too large an amount is used the manganese content in the finished steel may be lower than is desired. Also the cost may be unduly increased 40 because of undue loss of manganese and waste of siderite or its equivalent. I believe that there is a fairly well defined balance between the amounts of manganese present in metal form, and in non-metallic substances in steel and that when this 45 balance is disturbed there is a tendency for re-establishment of the balance. Consequently, it is important to know the manganese content before determining how much siderite or its equivalents to use. Knowledge of the amounts of 50 ingredients used to make a given steel and the manner in which the given steel was made are usually sufficient for this purpose and the making of a chemical analysis is not necessary.

Substances, other than siderite, which possess 55

the property of reducing the abrasiveness of the non-metallic substances in steel include iron oxide ores such as limonite, phosphate ores such as vivianite, and slow acting non-ferrous carbonates such as cerussite, rhodochrosite malachite and azurite. In general, any substance which will liberate oxygen or an oxygen containing gas in the molten steel rapidly, but not so rapidly as to result in an explosion, may be used. Combinations of two or more of these substances may be used. Although ores are mentioned because of their relatively low cost, substances which contain the oxygen compounds of these ores may be used satisfactorily. Sodium carbonate decomposes too rapidly for safe use, for it tends to explode and throw molten metal out of the ladle.

I believe that the treatment of steel with substances which decompose rapidly, but not too rapidly, in the steel, and liberate oxygen or an oxygen containing gas, bring about an oxidation of manganese and iron with resultant fluxing of the MnO with FeO and lowering of the fusing temperature; and that substances such as iron silicates, manganese silicates, iron manganese silicates, MnO, corresponding aluminates and other substances which are ordinarily relatively infusible, and therefore highly abrasive, are converted by such oxidizing or fluxing actions into more readily fusible substances, even into substances which melt at temperatures below the melting point of steel, with coincident decrease in abrasiveness. Moreover, I believe that the decrease in melting points of such substances with the agitation due to evolution of gas in the steel results in movement of considerable quantities of such substances into the slag, thus reducing the amount of such substances remaining in the steel when cold.

This invention is applicable to open hearth steels such as "killed" and "rimming" steels, steels having above about .80% of Mn, and steels in which the Mn is high to counteract high sulphur. This method may be carried out on open hearth steel with good results as follows: Tap the molten steel into a ladle, adding the predetermined amount of ferromanganese when the ladle

is about one-fourth filled and then add the calculated amount of siderite or other equivalent substances before slag covers the metal in the ladle. Alternatively, some of the manganese may be added in the furnace, if desired.

The invention is also of advantage with electric furnace steels. The metal is tapped while hot and the siderite or other equivalent is added in predetermined amount to the ladle during flow of the steel into the ladle.

Having thus described my invention so that those skilled in the art may understand and be able to practice the same, what I desire to secure by Letters Patent is defined in what is claimed.

What is claimed is:

1. The process of making steel which includes the steps of making Bessemer steel containing about .05% of manganese, adding about 1.25% of manganese to such steel while it is being poured into a ladle, and adding between about four and seven pounds of siderite per ton of steel to the steel during pouring into the ladle.

2. The process of making steel which includes the steps of making steel containing between about .80% and about 1.5% of manganese and non-metallic substances, and mixing with such steel, while molten, between about four pounds and about ten pounds of siderite per ton of steel.

3. The process of making steel which includes the steps of making, by the open hearth process, steel containing manganese and other non-metallic-substance-forming ingredients, adding manganese to such molten steel to bring the total manganese content of the steel to between about .80% and about 1.50%, and treating the molten steel with between about 4 pounds and about 10 pounds of siderite per ton of steel.

4. The process of making steel which includes the steps of making steel containing between about .80% and about 1.50% of manganese and non-metallic substances and mixing with such steel while molten between about 4 and about 10 pounds of an oxygen containing iron ore selected from the group consisting of siderite and limonite per ton of steel.

EARL C. SMITH.